

## 1

2,820,750

ELECTROLYTIC TREATMENT OF METALS  
AND ALLOYS

Percy Allan Charlesworth, Adlington, England

No Drawing. Application March 25, 1953  
Serial No. 344,670

5 Claims. (Cl. 204—140.5)

This invention relates to improvements in the electrolytic treatment of metal surfaces wherein an electrolyte comprising a mixture of sulphuric acid and phosphoric acid or sulphuric acid alone, the electrolyte being of high acid concentration, is employed and the article to be polished is made the anode.

In the specification of my U. S. Patent No. 2,594,124 an electrolytic polishing process is described having an electrolyte based on a mixture of sulphuric acid or phosphoric acid or on sulphuric acid alone to which is added a small amount of the aromatic amino compound, e. g. aniline.

I have now found and this discovery forms the basis of the present invention that stainless steel and other ferrous alloys with chromium and/or nickel; plain carbon steels and similar ferrous alloys; nickel and its alloys; chromium and its alloys and cobalt and its alloys can be satisfactorily electrolytically treated for the purpose of brightening, polishing, electro-machining, shaping, cutting and stress relieving or the like using an electrolyte based on a mixture of sulphuric acid and phosphoric acid or on sulphuric acid alone to which a relatively small amount of a heterocyclic compound or compounds of the type in which the heterocyclic molecule contains at least one ring structure having present in the ring at least two heterocyclic atoms one of which is nitrogen.

Although the invention is not limited thereto, I have found that it is particularly advantageous when the electrolyte has an acid concentration of at least 50% by weight of the electrolyte or more generally speaking has a combined sulphate and phosphate content which when expressed as sulphuric acid and phosphoric acid respectively represents at least 50% of the electrolyte and the ratio of sulphuric acid and phosphoric acid initially in the electrolyte exceeds 5:3.

The proportion of the additive necessary is small and falls within the range of 0.3% to 10% by weight of the electrolyte according to the particular additive or additives employed and the work the electrolyte is required to do.

Polishing processes using an electrolyte according to the present invention can be carried out using current densities within the range of 0.3 to 5 amps. per square inch. Higher current densities may be used for treatment requiring greater metal removal, e. g. electro-machining.

Generally a heterocyclic compound of the type referred to, to be satisfactory as an additive should satisfy the following requirements:

- (1) It should be effective at low concentrations, i. e. between 0.3% and 10% by weight of the electrolyte.
- (2) It should have a reasonable life.
- (3) Deleterious reaction products should be capable of removal from the electrolyte.
- (4) It should not cause excessive frothing or foaming nor give off malodorous or toxic vapors during the polishing process.

The following compounds are illustrative of the type of

## 5

## 2

molecular configuration of the additives: morpholine phenyl morpholine and thialidine, the structural formula of the latter compound being:



10 A compound may be used alone as the additive or two or more such compounds may be used together. Alternatively the heterocyclic compound or compounds may be used together with an aromatic amino compound such as aniline or with any other desired compound.

15 The following examples are illustrative of the invention, in each example the electrolyte having the initial composition:

## Parts by weight

|                                  |          |
|----------------------------------|----------|
| 20 $\text{H}_2\text{SO}_4$ ----- | 5        |
| $\text{H}_3\text{PO}_4$ -----    | 2        |
| $\text{H}_2\text{O}$ -----       | 15 to 30 |
| Morpholine -----                 | 2 to 10  |

Example 1.—*Stainless steel*.—A current density of 1 amp. per square inch and a temperature of 50–60° C.

25 Example 2.—*Plain carbon steels and low alloy steels*.—A current density of 1 amp. per square inch and a temperature of 85° C.

Example 3.—*Stainless iron, e. g. ferrous alloys having 17% chromium content*.—A current density of 1 amp. per square inch and a temperature of 85° C.

30 Example 4.—*An alloy in which the proportions of the main constituents are Ni—55%, Cr—20%, Co—20% e. g. Nimonic "90."*.—A current density of 1.8 amps. per square inch and a temperature of 30° C.

Example 5.—*An alloy in which the proportions of the main constituents are Ni—75%, Cr—20%, e. g. Nimonic "80."*.—A current density of 2.0 amps. per square inch and a temperature of 30° C.

35 Example 6.—*An alloy in which the proportion of the main constituents are Ni—70%, Cr—20%.*.—A current density of 1.0 amp. per square inch and a temperature of 30° C.

The additives and processing conditions employed are related to the metal or alloy being treated and the result desired. The time of treatment depends on the amount of metal to be removed; thus for polishing the time taken in the foregoing examples would be about 10 minutes whilst for machining it might be 30 minutes or longer.

40 Further the current density employed can also be varied according to the amount of metal to be removed.

The water and metal content of the electrolyte depends on its particular application and various forms of agitation may be employed as required.

45 55 I claim:

1. A method of anodically removing metal from the surface of a metallic body belonging to the group consisting of iron, nickel, chromium, cobalt and alloys of each, characterized by immersing at least a surface portion of said metallic body in an electrolyte solution containing at least 50% by weight of said solution of acid constituents belonging to the group consisting of sulphuric acid and of a mixture of sulphuric and phosphoric acid, the ratio of sulphuric acid in said mixture to phosphoric acid being greater than 5 to 3, said electrolyte solution also containing between 0.3% and 10% by weight of said solution of an additive belonging to the group consisting of morpholine and morpholine derivatives; and passing current through said metallic body and said electrolyte solution.
2. A method of anodically removing metal from the surface of a metallic body belonging to the group consist-

ng of iron, nickel, chromium, cobalt and alloys of each, characterized by immersing at least a surface portion of said metallic body in an electrolyte solution containing at least 50% by weight of said solution of acid constituents belonging to the group consisting of sulphuric acid and of a mixture of sulphuric and phosphoric acid, the ratio of sulphuric acid in said mixture to phosphoric acid being greater than 5 to 3, said electrolyte solution also containing between 0.3% and 10% by weight of said solution of morpholine; and passing current through said metallic body and said electrolyte solution.

3. A method of anodically removing metal from the surface of a metallic body belonging to the group consisting of iron, nickel, chromium, cobalt and alloys of each, characterized by immersing at least a surface portion of said metallic body in an electrolyte solution containing at least 50% by weight of said solution of acid constituents belonging to the group consisting of sulphuric acid and of a mixture of sulphuric and phosphoric acid, the ratio of sulphuric acid in said mixture to phosphoric acid being greater than 5 to 3, said electrolyte solution also containing between 0.3% and 10% by weight of said solution of phenyl morpholine; and passing current through said metallic body and said electrolyte solution.

4. A method of anodically removing metal from the surface of a metallic body belonging to the group consisting of iron, nickel, chromium, cobalt and alloys of each, characterized by immersing at least a surface portion of said metallic body in an electrolyte solution containing at least 50% by weight of said solution of acid constituents

belonging to the group consisting of sulphuric acid and of a mixture of sulphuric and phosphoric acid, the ratio of sulphuric acid in said mixture to phosphoric acid being greater than 5 to 3, said electrolyte solution also containing between 0.3% and 10% by weight of said solution of thialdine; and passing current through said metallic body and said electrolyte solution.

5. A method of anodically removing metal from the surface of a metallic body belonging to the group consisting of iron, nickel, chromium, cobalt and alloys of each, characterized by immersing at least a surface portion of said metallic body in an electrolyte solution containing at least 50% by weight of said solution of sulphuric acid, said electrolyte solution also containing between 0.3% and 10% by weight of said solution of an additive belonging to the group consisting of morpholine and morpholine derivatives; and passing current through said metallic body and said electrolyte solution.

#### References Cited in the file of this patent

##### UNITED STATES PATENTS

|           |              |               |
|-----------|--------------|---------------|
| 2,349,843 | Beckwith     | May 30, 1944  |
| 2,411,410 | Beckwith     | Nov. 19, 1946 |
| 2,451,341 | Jernstedt    | Oct. 12, 1948 |
| 2,594,124 | Charlesworth | Apr. 22, 1952 |
| 2,700,020 | Pierce       | Jan. 18, 1955 |

##### FOREIGN PATENTS

|         |               |              |
|---------|---------------|--------------|
| 683,310 | Great Britain | Nov. 6, 1952 |
|---------|---------------|--------------|